

## UNITED STATES PATENT OFFICE

2,096,318

METHOD OF MAKING CHROMIUM STEEL  
FROM CHROMIUM STEEL SCRAPVere B. Browne, Brackenridge, Pa., assignor to  
Allegheny Steel Company, a corporation of  
PennsylvaniaNo Drawing. Application January 31, 1936,  
Serial No. 61,805

7 Claims. (Cl. 75—12)

My present invention relates to the manufacture of chromium steels and more particularly to the manufacture of chromium steels and/or chromium-containing steels from steel scrap containing chromium.

The uses of chromium and chromium-containing steels, e. g., stainless steels, oxidation resistant steels, etc., have been rapidly increasing the past few years and bid fair to find application to an even greater extent in the future. Many articles have been and are being fabricated from these chromium steels with the result that large quantities of chromium steel scrap have accumulated due to the fact that the fabricating operations produce from about 40 to 50% of scrap.

This not only makes chromium steel and articles fabricated from chromium steel more expensive than they need be, but this scrap represents a serious economic loss.

Most chromium steels, at least those containing the higher amounts of chromium, are made in an electric arc furnace using carbon arcs. As a result, it is difficult to make these chromium steels low in carbon because chromium and carbon have a great affinity for each other. The fact that the carbon specification in these chromium steels must be low makes it necessary at the present time to use relatively expensive low carbon alloying materials such as low carbon ferro-chrome to obtain the desired chromium content in the steel or to go to the expense of using chromite ore and directly reducing it into the steel.

Despite the relatively large demand for chromium steels and articles fabricated therefrom no simple, economical and sure way has been developed to make them inexpensively or to utilize chromium steel scrap in making low carbon chromium steels and articles fabricated from. The accumulations of scrap, therefore, have relatively little use. If these scrap materials could be utilized to make first-quality, high-grade chromium steels such as are made by present methods, it would be possible not only to make these steels at materially lower cost, but their uses would be more widely distributed and certain applications could be taken advantage of at these lower costs, wherein chromium steels have not so far been able to be used. Moreover, the economic loss of the chromium steel scrap could be substantially entirely eliminated.

The method of my present invention enables me to make first-quality, high-grade chromium and/or chromium-containing steels in which there is incorporated relatively large percentages of chromium steel scrap material. I have found, for example, that I can incorporate anywhere from 40 or 50% up to about 70% or more of chromium-containing steel scrap and still produce chromium steel of the very highest quality.

While in general my new process relates to all chromium steels and/or chromium-containing steels, I have found that in particular three types of chromium steel can be readily and economically produced in accordance with my present method. I refer in this connection especially to chromium alloy steels containing about 18% chromium, about 13% chromium, and about 4-6% chromium. These particular chromium steels are today widely used and manufactured by various processes but by my present method I can produce them equally well and at materially decreased cost by utilizing chromium steel scrap of proper composition, due regard being given to the particular steel being made.

It is, therefore, one of the objects of my present invention to provide a method of making first-quality, high-grade chromium steels by utilizing considerable percentages of scrap steel containing chromium.

Another object resides in making low carbon chromium steels in which up to 70% or more of chromium steel scrap can be used in a given furnace charge.

An additional and more specific object resides in first producing a molten bath of steel containing no chromium, adjusting the carbon content thereof to a low figure and then incrementally adding chromium steel scrap and low-carbon ferro-chrome, where necessary, sufficient to adjust the chromium content of the whole to the desired figure.

Those skilled in this art will appreciate the further objects and advantages which are suggested by the present description or which will be understood therefrom.

In carrying out my present process, I first melt down a predetermined percentage of mild carbon steel or ordinary steel scrap to form a molten bath of suitable weight. I then refine the same under an oxidizing slag until I have reduced the carbon content to approximately .03%. When suitable test or analysis shows that the carbon content is approximately .03%, I remove the oxidizing slag from the molten bath of iron and I deoxidize and degasify it in accordance with the process set forth in my Patent No. 1,658,879. When this process is completed, the low carbon iron is covered and protected by a thin but voluminous calcium aluminate slag which not only protects the iron from carbon absorption and oxidation, but at the same time forms a reception slag for the chromium steel scrap which is thereafter incrementally added.

I now add incrementally to the low-carbon molten iron bath with the protective and reception slag thereon—and the operations may be carried out successfully in an electric arc furnace—chromium and/or chromium-containing steel scrap which has a carbon content insufficient to in-

crease the total carbon content of the final bath above the required carbon specification. Each incremental addition of chromium steel scrap is made in such manner that at first it floats partly submerged in the slag and thus burns off any carbonaceous matter with which the scrap might be contaminated before each such incremental addition becomes completely submerged in the protective slag. Such submergence is allowed to take place before power is applied. During these operations, the volume and viscosity of the slag is maintained by suitable additions of fluxing reagents such as alumina, fluorspar, etc. Upon the completion of these operations, I may thereafter add in the same manner, enough low-carbon ferro-chrome to adjust the total chromium content and any other alloying elements which are desired to be incorporated in the ultimate steel and in this way I accomplish the objects and advantages above outlined. Each of these additions is made in the same manner as the chromium steel scrap additions.

I may, for example, make suitable alloying additions such as tungsten, molybdenum, and any other desired element. In each case the additional alloying element is added in such form that it introduces no undesirable ingredients into the steel and also in such form that it does not result in increasing the carbon content beyond the permissible amount.

While I have made it possible to carry out these operations in an electric arc furnace—and I prefer to use such—it will be understood by those skilled in this art that my initial charge of low-carbon iron may be secured by transferring hot metal of the proper composition either from a Bessemer converter or from an open hearth furnace and that thereafter the process is carried out as explained above.

While I prefer to use a calcium aluminate slag and to reduce the iron with aluminum, I may, however, use any suitable slag forming materials such as lime and fluorspar, or lime and sand, and I may also make use of any suitable or desired reducing agent such as silicon or carbon to deoxidize the bath and to form the reception slag for the scrap additions.

While my process is particularly applicable and valuable in the production of chromium steels containing in the neighborhood of .10% carbon, or less, my process can, however, be also applied with advantage to the production of chromium steels in which a more liberal carbon specification is permissible. As already noted, chromium steels containing in the neighborhood of .10% carbon are perhaps the most valuable and at the same time the most difficult to make so that my process is of peculiar importance and value in connection with such steels.

I do not specifically claim, in this application, the manufacture of chromium nickel steels of the 18% chromium, 8% nickel type; such have been claimed in my copending application Serial No. 624,348 filed July 23, 1932.

What I claim as new and desire to secure by Letters Patent is:

1. In a method of the kind described, melting down a predetermined percentage of steel scrap, refining the same under an oxidizing slag until the carbon content thereof is reduced to about 0.03%, removing the slag, deoxidizing and degassing the molten metal, adding a calcium aluminate slag, incrementally adding chromium-containing steel scrap in predetermined amount, and

bringing the alloying elements of the whole up to the desired content.

2. In a method of the kind described, melting down a predetermined percentage of steel scrap in an electric furnace of the arc type, refining the same until its carbon content is about 0.03%, deoxidizing and degassing the molten metal, covering the molten metal with suitable slag forming materials, incrementally adding a predetermined amount of chromium-containing alloy steel scrap, and finally adjusting the alloy content of the whole by appropriate additions of alloying elements.

3. In a method of the kind described, melting down a predetermined percentage of steel scrap, refining the same until its carbon content is about 0.03%, deoxidizing and degassing the molten metal, covering the molten metal with suitable slag forming materials, incrementally adding a predetermined amount of chromium-containing alloy steel scrap, and finally adjusting the alloy content of the whole by appropriate additions of alloying elements, said slag forming materials being calcium aluminate.

4. In a method of the kind described, melting down a predetermined percentage of steel scrap in an electric furnace of the arc type, refining the same until its carbon content is about 0.03%, deoxidizing and degassing the molten metal, covering the molten metal with suitable slag forming materials, incrementally adding a predetermined amount of chromium-containing alloy steel scrap, and finally adjusting the alloy content of the whole by appropriate additions of alloying elements, said slag forming materials being lime and fluorspar.

5. In a method of the kind described, melting down a predetermined percentage of steel scrap in an electric furnace of the arc type, refining the same until its carbon content is about 0.03%, deoxidizing and degassing the molten metal, covering the molten metal with suitable slag forming materials, incrementally adding a predetermined amount of chromium-containing alloy steel scrap, and finally adjusting the alloy content of the whole by appropriate additions of alloying elements, said slag forming materials being lime and sand.

6. In a method of the kind described, forming a bath of molten steel, refining the same until the carbon content is lowered to approximately 0.03%, removing the slag formed by the foregoing, so treating the low carbon molten iron thus produced as to deoxidize and degasify the same and to form a calcium aluminate reception slag thereon, incrementally charging portions of chromium-containing steel scrap onto such reception slag, while suitably maintaining the volume and viscosity of the slag.

7. A method of making chromium steel containing about 18 per cent chromium and about .10 per cent carbon, with the remainder substantially all iron, from chromium steel scrap comprising forming a molten bath of carbon steel substantially free from chromium, reducing the carbon content of such bath to about .03 per cent, reducing oxide and gaseous contents of the bath to a low value, forming a calcium aluminate covering slag on said bath, incrementally adding chromium alloy steel scrap of approximately the ultimate analysis desired and adjusting the composition of the bath by appropriate low carbon ferro-chrome additions.

VERE B. BROWNE.